# EUROPEAN PATENT SPECIFICATION

(11) **EP 1 600 522 B1**
(45) Date of publication and mention of the grant of the patent: **16.12.2009**
(21) Application number: 05252324.8
(22) Date of filing: 14.04.2005
(51) Int. Cl.: C23C 4/00

(54) **Method of producing a self supporting form from a coating material**
Verfahren zur Herstellung einer selbsttragenden Form aus Beschichtungsmaterial
Procédé de fabrication d'une forme autoporteuse à partir d'un matériau de revêtement

(30) Priority: 29.05.2004 GB 0412097
(43) Date of publication of application: 30.11.2005
(73) Proprietor: ROLLS-ROYCE PLC, London, SW1E 6AT (GB)
(72) Inventor: Hopkins, Noel Paul, Derby DE23 4AR (GB); Shipton, Mark Henry, Bristol BS15 1XJ (GB)
(74) Representative: Gunn, Michael Alan

(56) References cited:
- EP-A- 1 072 692
- DD-A1- 280 823
- GB-A- 769 466
- GB-A- 827 266
- GB-A- 2 007 129
- REJDA E.F., SOCIE D.F.: "Bulk Property Evaluation of a Thick Thermal Barrier Coating" FATIGUE AND FRACTURE MECHANICS, 2000, - 2000 pages 143-163, XP008050948 astm stp 1389, G.Halford,American Society for Testing and Materials,West Conshohocken,PA
- PATENT ABSTRACTS OF JAPAN vol. 013, no. 111 (C-577), 16 March 1989 (1989-03-16) & JP 63 286563 A (YAMAKI KOGYO KK), 24 November 1988 (1988-11-24)
- Y. SUGA, D. LIAN AND S. KURIHARA: "Detection of Delamination of Sprayed Ceramic Coating in Thermal Schock Test by Ultrasonic Testing Method" PROCEEDINGS OF ITSC, May 1995 (1995-05), XP008050947 Kobe,Jp
- PATENT ABSTRACTS OF JAPAN vol. 2002, no. 11, 6 November 2002 (2002-11-06) & JP 2002 214123 A (ISHIKAWAJIMA HARIMA HEAVY IND CO LTD), 31 July 2002 (2002-07-31)

## Description

Coating materials are used to cover the surfaces of metallic objects, so as to protect the objects from degradation when subjected to hostile working conditions. An example of such objects are the turbine blades that operate in a gas turbine engine.

It is the practise in some designs, to make turbine blades from a given material, and coat their aerofoil portions with another material more able to withstand the high temperature gases that flow over them. The coating layer is usually a metal alloy and is normally applied by the know technique of thermal spraying and is very thin. It is important to have some idea of the structural integrity of the coating itself, and the quality of its adhesion to the blades aerofoils prior to actual use thereon.

There are a number of difficulties when trying to obtain material data from coatings. Firstly coatings are generally too thin to gain useful results when the coating is attached to a substrate. Secondly the substrate can often be stronger and/or stiffer than the coating and the effects of the substrate contaminate the test results. Thirdly the coating produced by thermal spraying has a particulate structure with different properties to cast materials of the same composition, thus it is not possible to look up material data from a data book of predetermined compositions. Fourthly the coating itself may be composite material with complex properties, eg a mixture of metal and ceramic.

When making a coating test piece, it is known to provide a salt based flat slab, and to thermally spray a particulate coating material on to one of its surfaces. On contact with the target surface, the particle cool rapidly and contract. Molten particles following and contacting the semi cooled particles generate residual stresses in the coating material. If as some times happens, the bond between the coating and the slab is not sufficiently strong, the coating de-laminates. Further if the slab is not sufficiently stiff, again as sometimes happens, the aforementioned residual stresses can induce distortion in the coating and slab. The resulting poor quality coating layer, when removed from the slab has too frequently proved unable to maintain an integral self supporting form that would give sufficiently accurate indication of strength when stressed on a standard mechanical test machine.

Rejda E.F, Socie D.F & Nuel B.P. "Bulk Property Evaluation of a Thick Thermal Barrier Coating" Fatigue & Fracture Mechanics, 31st Volume, ASTM STP 1389, G.R Halford & J.P Gallagher, Eds, American Society for Testing Materials, West Conshohocken, PA, 2000, pp 143-161 discloses producing a bulk coating material of 24% ceria-zirconia by spraying the ceramic powder onto a mild steel disk. The disk was etched away in nitric acid leaving a freestanding coating. The freestanding coating was sectioned into long strips using a low-speed diamond saw and epoxied to grooved copper blocks and this assembly was cut into sections of desired thickness and mounting holes were drilled for specimen gripping and each sample was ground using a low speed diamond grinder to final specimen shape.

GB2007129A discloses applying a metal or alloy coating to a workpiece or replica of a workpiece by gas atomising a stream of molten metal into particles to form a coating on the workpiece or replica of the workpiece. The coating remains on the workpiece or is removed and subsequently reapplied. The coating is removed from the replica of the workpiece and secured to the workpiece and the replica is reused.

The present invention seeks to provide an improved method of producing an integral self supporting form from particulate material.

According to the present invention a method of producing an integral self supporting test coating from particulate material comprises the steps of making a dissolvable mould having a depression therein which conforms to the desired shape and volume of said test coating, thermally spraying said particulate material into said depression on the dissolvable mould so as to overfill it, removing the excess material when solidified from the dissolvable mould so as to make the resulting exposed material surface flush with the relevant surface of said dissolvable mould, then dissolving the dissolvable mould away from the solidified test coating, utilising a dissolvable plastic, or plaster, to form the dissolvable mould, forming the dissolvable mould from a plastic, or plaster, that is dissolvable in water.

The invention will now be described by way of example and with reference to the accompanying drawings, in which;
Figure 1 is a pictorial view of a mould in accordance with the present invention.
Figure 2 is a pictorial view of an integral self supporting test piece formed in the mould of Figure 1.
Figure 3 is a view of the test pieces of Figure 2 in situ in a mechanical test rig.

Referring to Figure 1 a sacrificial mould 10 has a depression 12 of a desired shape and depth formed in a surface 14. In the present example, a test piece 16 (Figure 2) is produced by thermally spraying particles of molten metal into the depression 14. Spraying is performed long enough to overfill the depression 14, and when the metal has solidified, the excess is machined off so as to leave the exposed metal surface (not shown in Figure 1) flush with the outer surface of the mould.

Sacrificial mould 10 is made from a dissolvable plaster that on completion of the thermal spraying and machining operations, can be placed in water, and dissolved away from test piece 16.

Alternatively the sacrificial mould 10 may be made from a dissolvable plastic, or dissolvable plastic composite, that on completion of the flame spraying and machining operations, can be placed in water and dissolved away from test piece 16. A suitable plastic is sold under the trade name AQUAPOUR.

A thermally sprayed coating test piece, when made by the moulding process described, illustrated and claimed in this specification, is more robust than hitherto, by virtue of the walls of the mould containing the sprayed coating and restricting the affect that the residual stresses have on the sprayed coating. The mould also allows the coating to be sprayed to near net shape, reducing the amount of subsequent machining. A consequence is that a coating test piece can be more easily handled, and when mechanically stressed on a standard mechanical testing machine 18, provides more reliable information regarding the strength of the coating.

The method of producing integral self supporting test coating may be used to produce a number of test coatings with different dimensions and/or shapes for mechanically testing, for example tensile testing, fatigue testing, creep testing or CT testing to obtain data, eg to measure, the tensile, fatigue, creep and CT properties and performance characteristics of the coating material. The mechanical testing may be used to determine Young's Modulus at one or more temperatures for each coating material, test coating, tested.

The present invention is applicable to the production of integral self supporting test coatings by any thermal spraying technique, for example plasma spraying, flame spraying, combustion spraying, HVOF spraying etc. The present invention is applicable to various coatings for example thermal barrier coatings, eg zirconia or yttria stabilised zirconia, or other suitable ceramics, metal bond coatings and environmental protective coatings, eg metal or alloys McrAlY, McrAl, wear erosion resistant coatings, eg WC and/or abradable coatings, composite of metal and ceramic.

## Claims

1. A method of producing an integral self supporting test coating (16) from particulate material comprises the steps of (i) making a dissolvable mould (10) having a depression (12) therein which conforms to the desired shape and volume of said test coating (16), (ii) thermally spraying said particulate material into said depression (12) in the dissolvable mould (10) so as to overfill it, (iii) removing the excess material when solidified from the dissolvable mould (10) so as to make the exposed material surface flush with the relevant surface of said dissolvable mould (10), (iv) then dissolving the dissolvable mould (10) away from the solidified test coating (16) utilising a dissolvable plastic, or plaster, to form the dissolvable mould (10), forming the dissolvable mould (10) from a plastic, or plaster, that is dissolvable in water.

2. A method of producing an integral self supporting test coating (16) from particulate material as claimed in claim 1 including the step of utilising a plastic composite to form the dissolvable mould (10).

3. A method of producing an integral self supporting test coating (16) from particulate material as claimed in claim 1 or claim 2, including the step of plasma spraying, flame spraying, combustion spraying or HVOF spraying.

4. A method of producing an integral self supporting test coating (16) from particulate material as claimed in any of claims 1 to 3 wherein the particulate material comprises a metal, an alloy, a ceramic or a composite of metal and ceramic.

5. A method of producing an integral self supporting test coating (16) from particulate material as claimed in any of claims 1 to 4 wherein the test coating (16) comprises a thermal barrier coating, an environmental protective coating, a wear resistant coating or an abradable coating.

6. Use of an integral self supporting test coating (16) from particulate material as claimed in any of claims 1 to 5 for mechanically testing the integral self supporting test coating (16) to determine the mechanical properties of the coating material.

7. Use of an integral self supporting test coating (16) from particulate material as claimed in claim 6 wherein the mechanical testing comprises tensile testing, fatigue testing, creep testing or CT testing.

## Patentansprüche

1. Verfahren zur Herstellung eines integralen selbsttragenden Testkörpers (16) aus einem partikelförmigen Beschichtungsmaterial mit den folgenden Schritten: (i) es wird eine auflösbare Form (10) mit einer der Gestalt und dem Volumen des Testkörpers (16) entsprechenden Vertiefung (12) hergestellt; (ii) es wird das partikelförmige Beschichtungsmaterial in die Vertiefung (12) der auflösbaren Form (10) thermisch derart eingespritzt, dass sie übervoll wird; (iii) es wird das überschüssige Material nach seiner Erstarrung aus der auflösbaren Form (10) derart entfernt, dass die freiliegende Materialoberfläche mit der relevanten Oberfläche der auflösbaren Form (10) fluchtet; (iv) es wird dann die auflösbare Form (10) von dem erstarrten Testkörper (16) abgelöst, wobei ein auflösbares Plastikmaterial oder ein Plaster benutzt werden, um die auflösbare Form (10) zu erzeugen, und wobei die auflösbare Form (10) aus einem Plastikmaterial oder einem Plaster besteht, die in Wasser löslich sind.

2. Verfahren zur Herstellung eines integralen selbsttragenden Testkörpers (16) aus einem partikelförmigen Beschichtungsmaterial nach Anspruch 1, bei welchem ein Plastikverbundmaterial benutzt wird, um die auflösbare Form (10) herzustellen.

3. Verfahren zur Herstellung eines integralen selbsttragenden Testkörpers (16) aus einem partikelförmigen Beschichtungsmaterial nach den Ansprüchen 1 und 2, bei welchem ein Plasmaspritzen oder ein Flammspritzen oder ein Brennspritzen oder ein Hochgeschwindigkeits-Flammspritzen benutzt wird.

4. Verfahren zur Herstellung eines integralen selbsttragenden Testkörpers (16) aus einem partikelförmigen Beschichtungsmaterial nach einem der Ansprüche 1 bis 3, bei welchem das partikelförmige Beschichtungsmaterial aus Metall oder aus einer Legierung oder aus einem Keramikmaterial oder aus einem Verbundmaterial aus Metall und Keramik besteht.

5. Verfahren zur Herstellung eines integralen selbsttragenden Testkörpers (16) aus einem partikelförmigen Beschichtungsmaterial nach einem der Ansprüche 1 bis 4, bei welchem der Testkörper (16) aus einer thermischen Schutzschicht oder aus einer Umgebungsschutzschicht oder aus einer abnutzungsfreien Beschichtung oder aus einer abriebfesten Beschichtung besteht.

6. Benutzung eines integralen selbsttragenden Testkörpers (16) aus partikelförmigem Beschichtungsmaterial nach einem der Ansprüche 1 bis 5 zur mechanischen Prüfung des integralen selbsttragenden Testkörpers (16) aus Beschichtungsmaterial und zur Bestimmung der mechanischen Eigenschaften des Beschichtungsmaterials.

7. Benutzung eines integralen selbsttragenden Testkörpers (16) aus partikelförmigem Beschichtungsmaterial nach Anspruch 6, bei der die mechanische Prüfung einen Zugversuch, einen Ermüdungsversuch, einen Kriech-Dehnungs-Versuch oder einen Computertomographie-Versuch umfasst.

## Revendications

1. Procédé pour produire un revêtement de test autoporteur intégral (16) à partir d'un matériau particulaire comprenant les étapes consistant à (i) réaliser un moule soluble (10) ayant une dépression (12) à l'intérieur de celui-ci qui se conforme à la forme et au volume souhaités dudit revêtement de test (16), (ii) pulvériser thermiquement ledit matériau particulaire dans ladite dépression (12) dans le moule soluble (10) afin de trop le remplir, (iii) retirer le matériau en excès lorsqu'il est solidifié du moule soluble (10) afin de mettre la surface de matériau exposée de niveau avec la surface appropriée dudit moule soluble (10), (iv) dissoudre ensuite le moule soluble (10) pour l'éloigner du revêtement de test (16) solidifié en utilisant un plastique ou un plâtre soluble pour former le moule soluble (10), former le moule soluble (10) à partir d'un plastique ou du plâtre qui est soluble dans l'eau.

2. Procédé pour produire un revêtement de test autoporteur intégral (16) à partir d'un matériau particulaire selon la revendication 1, comprenant l'étape consistant à utiliser un composite de plastique pour former le moule soluble (10).

3. Procédé pour produire un revêtement de test autoporteur intégral (16) à partir d'un matériau particulaire selon la revendication 1 ou la revendication 2, comprenant l'étape de projection au plasma, à la flamme, à la combustion ou de projection HVOF.

4. Procédé pour produire un revêtement de test autoporteur intégral (16) à partir d'un matériau particulaire selon l'une quelconque des revendications 1 à 3, dans lequel le matériau particulaire comprend un métal, un alliage, une céramique ou un composite de métal et de céramique.

5. Procédé pour produire un revêtement de test autoporteur intégral (16) à partir d'un matériau particulaire selon l'une quelconque des revendications 1 à 4, dans lequel le revêtement de test (16) comprend un revêtement de barrière thermique, un revêtement de protection environnementale, un revêtement résistant à l'usure ou un revêtement pouvant être abrasé.

6. Utilisation d'un revêtement de test autoporteur intégral (16) à partir d'un matériau particulaire selon l'une quelconque des revendications 1 à 5, pour tester mécaniquement le revêtement de test autoporteur solidaire (16) afin de déterminer les propriétés mécaniques du matériau de revêtement.

7. Utilisation d'un revêtement de test autoporteur solidaire (16) à partir d'un matériau particulaire selon la revendication 6, dans laquelle le test mécanique comprend le test à la traction, le test à la fatigue, le test au fluage ou le test CT.
